# EUROPEAN PATENT SPECIFICATION

(11) **EP 0 429 240 B1**
(45) Date of publication and mention of the grant of the patent: **27.03.1996**
(21) Application number: 90312399.0
(22) Date of filing: 14.11.1990
(51) Int. Cl.: G03C 7/32, G03C 7/392

(54) **Silver halide photographic material**
Photographisches Silberhalogenidmaterial
Matériau photographique à l'halogénure d'argent

(30) Priority: 15.11.1989 JP 298092/89
(43) Date of publication of application: 29.05.1991
(73) Proprietor: KONICA CORPORATION, Tokyo 160 (JP)
(72) Inventor: Ogawa, Takahiro, Odawara-shi, Kanagawa-ken 250 (JP); Takada, Shun, Odawara-shi, Kanagawa-ken 250 (JP)
(74) Representative: Ellis-Jones, Patrick George Armine

(56) References cited:
- EP-A- 0 283 324
- EP-A- 0 330 093
- Patent Abstracts of Japan, vol. 9, no. 273 (P-401)[1996], October 30, 1985; & JP-A-60 119 547

## Description

### BACKGROUND OF THE INVENTION

This invention relates to a silver halide photographic material, more particularly to a silver halide photographic material that is capable of faithful color reproduction and that has improved raw stockstability.

Japanese Patent Application (kokai) No. 123047/1988 describes a silver halide photographic material containing a yellow coupler of the general formula (I) on a support. Japanese Patent Application (kokai) No. 231451/1988, which corresponds with EP-A-0283329, describes a silver halide photographic material containing on a support a yellow and a magenta coupler represented by the general formulas (I) and (II) and a phenolic cyan coupler having a substituent ethyl group on 3-position.

These conventional silver halide color photographic materials are capable of faithful color reproduction but it has been found that the use of the yellow coupler of the general formula (I) causes marked desensitization in raw stock during storage.

EP-A-0 330 093 describes a silver halide color photographic material containing at least one compound of the general formulae (I), (II), (III), and (IV) as an anti-bacterial agent.

### SUMMARY OF THE INVENTION

An object, therefore, of the present invention is to provide a silver halide photographic material that is capable of faithful color reproduction and which yet has good raw stock stability.

This object of the present invention can be attained by a silver halide color photographic material having on a support a yellow coupler represented by the following general formula (Y-I), a magenta coupler represented by the following general formula (M-I) and a cyan coupler represented by the following general formula (C-I), which photographic material is characterized by containing at least one of the compounds represented by the following general formulas (I), (II), (III) and (IV): where R₁ is an alkyl group, a cycloalkyl group or an aryl group; R₂ is an alkyl group, a cycloalkyl group, an aryl group or an acyl group; R₃ is an optional substituent on the benzene ring; n is 0 or 1; X₁ is a group capable of leaving upon coupling with the oxidation product of a developing agent; and Y₁ is an organic group; where Z is the nonmetallic group necessary to form a nitrogenous hetero ring which may optionally have a substituent; X is a hydrogen atom or a group capable of leaving upon reaction with the oxidation product of a color developing agent; and R is a hydrogen atom or a substituent; where R₁₁ is a ballast group; R₁₂ is an alkyl group having 2 or more carbon atoms; and Z₁ is a hydrogen atom or an atom or group that is capable of leaving upon reaction with the oxidation product of a color developing agent; where R₁₀ is a lower alkylene group; M is a hydrogen atom, an alkali metal or an alkyl group; X is a halogen atom, an alkyl group, a cycloalkyl group, an aryl group, a carboxyl group, an amino group, a hydroxyl group, a sulfo group, a nitro group or an alkoxycarbonyl group; n is 0 or 1; and m is an integer of 1 - 5 ; where R₂₀ is a hydrogen atom, an alkyl group, a cycloalkyl group, an alkenyl group, an aralkyl group, an aryl group, an alkoxy group, -CONHR (R is alkyl, aryl, alkylthio, arylthio, alkylsulfonyl or arylsulfonyl group) or a heterocyclic group; R₃₀ and R₄₀ are each a hydrogen atom, a halogen atom, an alkyl group, a cycloalkyl group, an aryl group, a heterocyclic group, a cyano group, an alkylthio group, an arylthio group, an alkylsulfoxide group, an alkylsulfonyl group, or an alkylsulfinyl group, provided that R₃₀ and R₄₀ may combine together to form an optionally substituted benzene ring; where R₅₀ and R₆₀ are each a hydrogen atom, a halogen atom, a lower alkyl group having 1 - 5 carbon atoms or a hydroxymethyl group; and R₇₀ is a hydrogen atom or a lower alkyl group having 1 - 5 carbon atoms; where R₈₀ is a hydrogen atom, an alkyl group or an aryl group; R₉₀ is a hydrogen atom, an alkyl group, an aryl group, an nitro group, a carboxyl group, a sulfo group, a sulfamoyl group, a hydroxy group, a halogen atom, an alkoxy group or a thiazolyl group; m is 0 or 1; and Z is the atomic group necessary to form a thiazolyl ring.

### DETAILED DESCRIPTION OF THE INVENTION

The present invention is described below in detail. The yellow coupler represented by the general formula (Y-I) Is first described. Examples of the alkyl group represented by R₁ in the general formula (Y-I) include methyl, ethyl, isopropyl, t-butyl and dodecyl. These alkyl groups may further contain substituents such as a halogen atom, an aryl group, an alkoxy group, an aryloxy group, an alkylsulfonyl group, an acylamino group and a hydroxy group.

Examples of the cyaloalkyl group represented by R₁ include a cyclopropyl group, a cyclohexyl group and an adamantyl group.

Examples of the aryl group represented by R₁ include a phenyl group.

A branched alkyl group is preferred as R₁.

The alkyl and cycloalkyl groups represented by R₂ in the general formula (Y-I) may be exemplified by the same groups as listed for R₁, and an illustrative aryl group is a phenyl group. The alkyl, cycloalkyl and aryl groups represented by R₂ may have the same substituents as in R₁. Examples of the acyl group represented by R₂ include an acetyl group, a propionyl group, a butyryl group, a hexanoyl group and a benzoyl group. An alkyl or aryl group is preferred as R₂, with an alkyl group being more preferred. A particularly preferred example of R₂ is a lower alkyl group having no more than 5 carbon atoms.

Examples of the optional substituent on the benzene ring which is represented by R₃ in the general formula (Y-I) include: a halogen atom (e.g. chlorine), an alkyl group (e.g. ethyl, i-propyl or t-butyl), an alkoxy group (e.g. methoxy), an aryloxy group (e.g. phenyloxy), an acyloxy group (e.g. methylcarbonyloxy or benzoyloxy), an acylamino group (e.g. acetamino or phenylcarbonylamino), a carbamoyl group (e.g. N-methylcarbamoyl or N-phenylcarbamoyl), an alkylsulfonamido group (e.g. ethylsulfonamido), an arylsulfonamido group (e.g. phenylsulfonamido), a sulfamoyl group (e.g. N-propylsulfamoyl or N-phenylsulfamoyl), and an imido group (e.g. succinylimido or glutarimido).

In the general formula (Y-I), Y₁ represents an organic group. While Y₁ is not limited in any other way, it is preferably a group represented by the following general formula (Y-II):${\text{- J - R}}_{\text{4}}$

In the general formula (Y-II), R₄ is an organic group containing one linkage group having a carbonyl or sulfonyl unit. Illustrative groups having a carbonyl unit include an ester group, an amido group, a carbamoyl group, a ureido group and a urethane group, and illustrative groups having a sulfonyl unit include a sulfonyl group, a sulfonamido group, a sulfamoyl group and an aminosulfonamido group. In the formula (Y-II), J is where R₅ is a hydrogen atom, an alkyl group, an aryl group or a heterocyclic group. Examples of the alkyl group represented by R₅ include methyl, ethyl, isopropyl, t-butyl and dodecyl, and examples of the aryl group represented by R₅ include phenyl and naphthyl.

The alkyl or aryl group represented by R₅ may have a substituent. While there is no particular limitation on the substituent, typical examples include: a halogen atom (e.g. chlorine), an alkyl group (e.g. ethyl or t-butyl), an aryl group (e.g. phenyl, p-methoxyphenyl or naphthyl), an alkoxy group (e.g. ethoxy or benzyloxy), an aryloxy group (e.g. phenoxy), an alkylthio group (e.g. ethylthio), an arylthio group (e.g. phenylthio), an alkylsulfonyl group (e.g. β-hydroxyethylsulfonyl), an arylsuflonyl (e.g. phenylsulfonyl), as well as an acylamino such as an alkylcarbonylamino (e.g. acetamido) or an arylcarbonylamino (e.g. phenylcarbonylamino). Other useful substituents include carbamoyl groups having an alkyl or aryl (preferably phenyl) as a substituent, such as an N-methylcarbamoyl group and an N-phenylcarbamoyl group. Also included are an alkylcarbonyl group such as acyl (e.g. acetyl) and an arylcarbonyl group such as benzoyl, as well as sulfonamido groups such as an alkylsulfonamido (e.g. methylsulfonamido) and an arylsulfonamido (e.g. benzenesulfonamido). Sulfamoyl groups having an alkyl or aryl (preferably phenyl) as a substituent can also be used as substituents and specific examples include N-methylsulfamoyl and N-phenylsulfamoyl groups. Also useful are a hydroxy group, a nitrile group, etc.

In the general formula (Y-I), x₁ represents a group capable of leaving upon coupling reaction with the oxidation product of a developing agent and may represent a group having the following general formula (Y-III) or (Y-IV), with the latter being preferred:${\text{- OR}}_{\text{6}}$ where R₆ is an optionally substituted aryl or heterocyclic group; where Z₁ represents the nonmetallic group necessary to form a 5- or 6-membered ring in conjunction with the nitrogen atom, as exemplified by methylene, methine, substituted methine, 〉C = 0, (R_{A} has the same meaning as R₅), -N=, -O-, -S- and -SO₂-.

The yellow coupler represented by the general formula (Y-I) may take on a his form, with two molecules bonded at site R₁, R₃ or Y₁.

Compounds represented by the following general formula (Y-V) are preferred yellow couplers for use in the present invention: where R₁, R₂, R₃ and J are the same as R₁, R₂ and R₃ in the general formula (Y-I) and J in the general formula (Y-II); n is 0 or 1; R₇ is an alkylene group, an arylene group, an alkylenearylene group, an arylenealkylene group or -A-V₁-B (where A and B are each an alkylene group, an arylene group, an alkylenearylene group or an arylenealkylene group; and V₁ is a divalent linkage group); R₈ is an alkyl group, a cycloalkyl group, an aryl group or a heterocyclic group; P is a bonding group having a carbonyl or sulfonyl unit; and X₁ is a group capable of leaving upon coupling with the oxidation product of a developing agent.

Examples of the alkylene group represented by R₇ in the general formula (Y-V) include a methylene group, an ethylene group, a propylene group, a butylene group and a hexylene group. These alkylene groups may have substituents such as an alkyl group, as in methyl-methylene, ethyl-ethylene, 1-methyl-ethylene, 1-methyl-2-ethyl-ethylene, 2-decyl-ethylene, 3-hexyl-propylene or 1-benzyl-ethylene, or an aryl group, as in 2-phenyl-ethylene or 3-naphthyl-propylene.

Examples of the arylene group represented by R₇ include a phenylene group and a naphthylene group.

Examples of the alkylarylene group represented by R₇ include a methylenephenylene group, and examples of the arylenealkylene group represented by R₇ include a phenylenemethylene group.

The alkylene group, arylene group, alkylenearylene and arylenealkylene groups represented by A and B are the same as the alkylene group, arylene group, alkylenearylene group and arylenealkylene groups represented by R₇ in the general formula (Y-V). Examples of the divalent linkage group represented by V₁ include groups such as -O- and -S-.

Among the alkylene, arylene, alkylenearylene and arylenealkylene groups and -A-V₁-B which are represented by R₇, an alkylene group is particularly preferred.

Examples of the alkyl group represented by R₈ in the general formula (Y-V) include an ethyl group, a butyl group, a hexyl group, an octyl group, a dodecyl group, a hexadecyl group and an octadecyl group. These alkyl groups may be straight or branched. Examples of the cycloalkyl group represented by R₈ include a cyclohexyl group. Examples of the aryl group represented by R₈ include a phenyl group and a napthyl group. Examples of the heterocyclic group represented by R₈ include a pyridyl group. These alkyl, cycloalkyl, aryl and heterocyclic groups represented by R₈ may contain substituents. Illustrative substituents are not limited in any way and may include the same substituents as listed for R₅, except that organic groups having a dissociative hydrogen atom having a pKa value of no more than 9.5 (e.g. a phenolic hydrogen atom) are not preferred as substituents in R₈.

In the general formula (Y-V). P represents a bonding group having a carbonyl or sulfonyl unit, preferably a group within the following class (Y-VI), more preferably a bonding group having a sulfonyl unit:

### Class (Y-VI):

and where R and R' which may be the same or different each represents a hydrogen atom, an alkyl group, an aryl group, or a heterocyclic group. Examples of the groups represented by R and R' may be the same as those listed for R₅. Those groups may have substituents which are the same as those listed for R₅. A hydrogen atom is preferred as R and R'.

The yellow coupler represented by the general formula (Y-I) is preferably used in an amount ranging from 1 x 10⁻³ to 1 mole, more preferably from 1 x 10⁻ to 8 x 10⁻¹ moles, per mole of silver halide.

The following are specific but non-limiting examples of the yellow coupler represented by the general formula (Y-I).

The magenta coupler represented by the general formula (M-I) is next described below.

In the general formula (M-I), Z represents the nonmetallic atomic group necessary to form a nitrogenous hetero ring which may have a substituent. In the formula (M-I), X represents a hydrogen atom or a group capable of leaving upon reaction with the oxidation product of a color developing agent. In the formula (M-I), R represents a hydrogen atom or a substituent. While there is no particular limitation on the substituent represented by R, typical examples include groups such as alkyl, aryl, anilino, acylamino, sulfonamido, alkylthio, arylthio, alkenyl and cycloalkyl. Other examples include: halogen, cycloalkenyl, alkynyl, hetero ring, sulfonyl, sulfinyl, phosphonyl, acyl, carbamoyl, sulfamoyl, cyano, alkoxy, aryloxy, heterocycloxy, siloxy, acyloxy, carbamoyloxy, amino, alkylamino, imido, ureido, sulfamoylamino, alkoxycarbonylamino, aryloxycarbonylamino, alkoxycarbonyl, aryloxycarbonyl and heterocyclic thio; as well as spiro compound residues and bridged hydrocarbon compound residues.

The alkyl group represented by R in the general formula (M-I) preferably contains 1 - 32 carbon atoms and it may be straight or branched.

The aryl group represented by R is preferably a phenyl group.

Examples of the acylamino group represented by R include alkylcarbonylamino and arylcarbonylamino.

Examples of the sulfonamido group represented by R include alkylsulfonamido and arylsulfonamido.

The alkyl and aryl moieties in the alkylthio and arylthio groups, respectively, represented by R may be the same as the alkyl and aryl groups listed above for R.

The alkenyl group represented by R preferably contains 2 - 32 carbon atoms, and the cycloalkyl group represented by R preferably contains 3 - 12 carbon atoms, more preferably 5 - 7 carbon atoms. The alkenyl group may be straight or branched.

The cycloalkenyl group represented by R preferably contains 3 - 12 carbon atoms, more preferably 5 - 7 carbon atoms.

Examples of the sulfonyl group represented by R include alkylsulfonyl and arylsulfonyl; examples of the sulfinyl group represented by R include alkylsulfinyl and arylsulfinyl; examples of the phosphonyl group represented by R include alkylphosphonyl, alkoxyphosphonyl, aryloxyphosphonyl and arylphosphonyl; examples of the acyl group represented by R include alkylcarbonyl and arylcarbonyl; examples of the carbamoyl group represented by R include alkylcarbamoyl and arylcarbamoyl; examples of the sulfamoyl group represented by R include alkylsulfamoyl and arylsulfamoyl; examples of the acyloxy group represented by R include alkylcarbonyloxy and arylcarbonyloxy; examples of the carbamoyloxy group represented by R include alkylcarbamoyloxy and arylcarbamoyloxy; examples of the ureido group represented by R include alkylureido and arylureido; examples of the sulfamoylamino group represented by R include alkylsulfamoylamino and arylsulfamoylamino; the heterocyclic group represented by R is preferably 5- to 7-membered and may be exemplified by 2-furyl, 2-thienyl, 2-pyrimidinyl and 2-benzothiazolyl; the heterocycloxy group represented by R preferably contains a 5- to 7-membered hetero ring and may be exemplified by 3,4,5,6-tetrahydropyranyl-2-oxy and 1-phenyltetrazol-5-oxy; the heterocyclic thio group represented by R is preferably a 5- to 7-membered heterocyclic thio group and may be exemplified by 2-pyridylthio, 2-benzothiazolylthio, and 2,4-diphenoxy-1,3,5-triazole-6-thio; examples of the siloxy group represented by R include trimethylsiloxy, triethylsiloxy and dimethylbutylsiloxy; examples of the imido group represented by R include succinimido, 3-heptadecylsuccinimido, phthalimido and glutarimido; an example of the spiro compound residue represented by R is spiro[3.3]heptan-1-yl; and examples of the bridged hydrocarbon compound residue represented by R include bicyclo[2.2.1]heptan-1-yl, tricyclo[3.3.1.1³.7]decan-1-yl, and 7,7-dimethyl-bicyclo[2.2.1]heptan-1-yl.

Examples of the group represented by X which is capable of leaving upon reaction with the oxidation product of a color developing agent include: a halogen atom (e.g. Cl, Br or F), as well as alkoxy, aryloxy, heterocycloxy, acyloxy, sulfonyloxy, alkoxycarbonyloxy, aryloxycarbonyl, alkyloxalyloxy, alkoxyoxalyloxy, alkylthio, arylthio, heterocyclic thio, alkyloxycarbonylthio, acylamino, sulfonamido, N-bound nitrogenous hetero ring, alkyloxycarbonylamino, aryloxycarbonylamino, carboxyl, and (where R₁′ has the same meaning as R; Z′ has the same meaning as Z; R₂′ and R₃′ each represents a hydrogen atom, an aryl group, an alkyl group or a heterocyclic group). Preferably, X is a halogen atom, especially a chlorine atom.

Examples of the nitrogenous hetero ring formed by Z or Z′ include a pyrazole ring, an imidazole ring, a triazole ring and a tetrazole ring. These rings may have substituents that are exemplified by those which are listed for R.

The compounds represented by the general formula (M-I) may be more specifically represented by the following general formulas (M-II) to (M-VII):

In the general formulas (M-II) to (M-VII), R₁ - R₈ and X have the same meanings as R and X. Among the compounds represented by the general formula (M-I), those which are represented by the following general formula (M-VIII) are particularly preferred: where R₁, X and Z₁ have the same meanings as defined for R, X and Z in the general formula (M-I).

Among the magenta couplers represented by the general formulas (M-II) to (M-VII), those which are represented by the general formula (M-II) are particularly preferred.

The substituents R and R₁ on the hetero ring described above are most preferably represented by the following general formula (M-IX): where R₉, R₁₀ and R₁₁ have the same meaning as R. Any two of R₉, R₁₀ and R₁₁, say, R₉ and R₁₀ may combine to form a saturated or unsaturated ring (e.g. cycloalkane, cycloalkene or hetero ring), and R₁₁ may further bind to said ring to form a bridged hydrocarbon compound residue.

Among the substituents represented by the general formula (M-IX), the following two cases are preferred: (i) where at least two of R₉ - R₁₁ are an alkyl group; and (ii) where at least one of R₉ - R₁₁, say R₁₁ is a hydrogen atom, with the other members, say, R₉ and R₁₀ combining to form a cycloalkyl together with the room carbon atoms, In case (i), it is particularly preferred if two of R₉ -R₁₁ is an alkyl group, with the other being a hydrogen atom or an alkyl group.

The ring that is formed by Z in the general formula (M-I), the substituent that may be possessed by the ring formed by Z₁ in the general formula (M-VIII), and R₂ - R₈ in the general formulas (M-II) to (M-VI) are preferably represented by the following general formula (M-X):${\text{- R}}^{\text{1}} {\text{- SO}}_{\text{2}} {\text{- R}}^{\text{2}}$ where R¹ is an alkylene group; and R is an alkyl group, a cycloalkyl group or an aryl group. The alkylene group represented by R¹ preferably contains at least two, more preferably 3 - 6, carbon atoms in the straight portion, and it may be either straight or branched. The cycloalkyl group represented by R is preferably 5- or 6-membered.

Typical but non-limiting examples of the magenta coupler represented by the general formula (M-I) are listed below.

Magenta couplers that can be used in the present invention in addition to the magenta couplers described above are the compounds identified under Nos. 1 - 4, 6, 8 - 17, 19 - 24, 26 - 43, 45 - 59, 61 - 104, 106 - 121, 123 - 162 and 164 - 223 on pages 66 - 122 in the specification of Japanese Patent Application No. 9791/1986.

The couplers described herein can be synthesized with reference being made to Journal of the Chemical Society, Perkin I (1977), 2047 - 2052, U.S. Patent No. 3,725,067, as well as Japanese Patent Application (kokai) Nos. 99437/1984, 42045/1983, 162548/1984, 171956/1984, 33552/1985, 43659/1985, 172982/1985 and 190770/1985.

The coupler of the general formula (M-I) can be used in amounts that preferably range from 1 x 10⁻³ to 1 mole, more preferably from 1 x 10⁻ to 8 x 10⁻¹ moles, per mole of silver halide.

The coupler of the general formula (M-I) may be used in combination with other magenta couplers.

The cyan coupler represented by the general formula (C-I) is now described below.

In the general formula (C-I), the alkyl group represented by R₁₂ may be straight or branched and it may optionally have a substituent. Preferably, R₁₂ is an alkyl group having 2 - 6 carbon atoms.

The ballast group represented by R₁₁ in the general formula (C-I) is an organic group having such a size and shape as to provide the coupler molecule with a sufficient degree of bulkiness to effectively prevent the coupler from diffusing from the layer where it is incorporated to another layer. This ballast group is preferably represented by the following general formula: where Rₙ₁ is an alkyl group having 1 - 12 carbon atoms, and Ar is an aryl group such as phenyl that may optionally contain a substituent.

The following are specific but non-limiting examples of the cyan coupler represented by the general formula (C-I).

Specific examples of these cyan couplers and others that can be used in the present invention are described in Japanese Patent Publication No. 11572/1974, as well as Japanese Patent Application (kokai) Nos. 3142/1976, 9652/1986, 9653/1986, 39045/1986, 50136/1986, 99141/1986, 105545/1986.

The cyan dye forming coupler represented by the general formula (C-I) can be used in amounts that preferably range from 1 x 10⁻³ to 1 mole, more preferably from 1 x 10⁻ to 8 x 10⁻¹ moles, per mole of silver halide.

It is preferable for the purpose of the present invention to use two cyan couplers in combination, the coupler represented by the formula (C-I) and a 2,5-diacylamino cyan coupler.

In the next place, the compounds of the general formulas (I), (II), (III) and (IV) which are additionally used in the present invention are described below.

In the general formula (I), the lower alkyl group represented by R₁₀ may be exemplified by methylene, ethylene and propylene. The halogen atom represented by X may be exemplified by chlorine, bromime or iodine. The alkyl group represented by X is preferably a straight or branched alkyl group having 1 - 8 carbon atoms. The cycloalkyl group represented by X is preferably a cycloalkyl group having 1 - 8 carbon atoms. The aryl group represented by X is preferably a phenyl or naphthyl group. The alkoxycarbonyl group preferably has 1 - 5 carbon atoms. Each of the groups listed above may have a substituent such as an alkyl group having 1 - 4 carbon atoms, a halogen atom, a hydroxyl group, a sulfo group, a nitro group, an amino group, a cyano group, a carboxyl group or a phenyl group.

The alkyl or alkenyl group represented by R₂₀ in the general formula (II) preferably has 1 - 36 carbon atoms, more preferably 1 - 18 carbon atoms. The cycloalkyl group represented by R₂₀ preferably has 3 - 12 carbon atoms, more preferably 3 - 6 carbon atoms. The alkyl, alkenyl, cycloalkyl, aralkyl, aryl and heterocyclic groups represented by R₂₀ may have substituents which are selected from among the following: a halogen atom, nitro, cyano, thiocyano, aryl, alkoxy, aryloxy, carboxy, sulfoxy, alkylcarbonyl, arylcarbonyl, alkoxycarbonyl, aryloxycarbonyl, sulfo, acyloxy, sulfamoyl, carbamoyl, acylamino, diacylamino, ureido, thioureido, urethane, thiourethane, sulfonamido, hetero ring, arylsulfonyloxy, alkylsulfonyloxy, arylsulfonyl, alkylsulfonyl, arylthio, alkylthio, alkylsulfinyl, arylsulfinyl, alkylamino, dialkylamino, anilini, N-alkylanilino, N-arylanilino, N-acylamino, hydroxy and mercapto.

The alkyl group represented by R₃₀ and R₄₀ in the general formula (II) preferably contains 1 - 18 carbon atoms, more preferably 1 - 9 carbon atoms. The cycloalkyl group represented by R₃₀ and R₄₀ preferably has 3 - 12 carbon atoms, more preferably 3 - 6 carbon atoms. The alkyl, cycloalkyl and aryl groups represented by R₃₀ and R₄₀ may have substituents such as halogen, nitro, sulfone, aryl and hydroxy. In the case where R₃₀ and R₄₀ combine to form a benzene ring, the benzene ring may have substituents such as hydrogen, halogen, alkyl, alkoxy, cyano and nitro.

The lower alkyl having 1 - 5 carbon atoms which is represented by R₅₀, R₆₀ and R₇₀ in the general formula (III) and the hydroxymethyl group represented by R₇₀ may have a substituent.

In the general formula (IV), R₈₀ is preferably a hydrogen atom; R₉₀ is preferably a hydrogen atom, an alkyl group having 1 - 3 carbon atoms, an amino group, a nitro group, a sulfo group, a halogen atom, or a hydroxy group; m is preferably 1; and the thiazolyl group represented by Z is preferably

Some of the compounds represented by the general formulas (I), (II), (III) and (IV) are known as preservatives for hydrophilic colloids in silver halide photographic materials. Part of the compounds represented by the general formula (I) are described in Japanese Patent Application (kokai) Nos. 22847/1984 and 257747/1988; part of the compounds represented by the general formula (II) are described in Japanese Patent Application (kokai) Nos. 27424/1979, 131929/1984, 142543/1984, 166343/1983, 131929/1984, 142543/1984 and 226343/1984; part of the compounds represented by the general formula (III) are described in Japanese Patent Application Nos. 119547/1985 and 231936/1987; and part of the compounds represented by the general formula (IV) are described in Japanese Patent Application (kokai) Nos. 274944/1988 and 263938/1985.

However, none of these references contain a single passage that teaches the effectiveness of the compounds (I) - (IV) in improving the raw stock stability of silver halide photographic materials.

Typical but by no means limiting examples of the compounds represented by the general formulas (I), (II), (III) and (IV) are listed below.

One or more members that are selected from among the compounds illustrated above may be used in the present invention. These compounds are well known in the art and are commercially available from ICI, Japan, Dainippon Ink & Chemicals, Inc., Rohm & Haas, Japan, San-ai oil Co., Ltd..

The amounts in which the compounds of the general formulas (I), (II), (III) and (IV) are used are not limited to any particular values but they are preferably in the range of 1 x 10⁻⁴ to 1 x 10⁻ g/m. Those compounds may be incorporated in either silver halide emulsion layers or non-emulsion layers or both. There also is no particular limitation on the method by which those compounds are added.

Compounds such as dye forming couplers to be used in the silver halide photographic material of the present invention are usually dissolved in high-boiling point (≥ca. 150°C) organic solvents or water-insoluble high-molecular weight compounds, optionally in combination with low-boiling point and/or water-insoluble organic solvents, and the resulting solutions are emulsified or dispersed in hydrophilic binders such as aqueous solutions of gelatin with the aid of surfactants, followed by addition to a hydrophilic colloidal layer of interest. In preparing dispersions, the low-boiling point organic solvent may be removed simultaneously with the step of dispersion.

The high-boiling point organic solvents to be used in the present invention are preferably those compounds which have dielectric constants of no more than 6.5 and which may be exemplified by esters (e.g. phthalate esters and phosphate esters), organic acid amides, ketones and hydrocarbon compounds that have dielectric constants of no more than 6.5. More preferred are those high-boiling point organic solvents which have dielectric constants of 1.9 - 6.5 and vapor pressures of up to 0.5 mmHg at 100°C. Among those organic solvents, phthalate esters and phosphate esters are particularly preferred. The most preferred are dialkyl phthalates having an alkyl group with at least 9 carbon atoms. Two or more high-boiling point organic solvents may be used in admixture. The term "dielectric constant" means a dielectric constant at 30°C.

The high-boiling point organic solvents described above are generally used in amounts ranging from 0 to 400 wt% of coupler, preferably from 10 to 100 wt% of coupler.

The silver halide photographic material of the present invention may be a color negative or positive film or a color paper. The advantage of the present invention is particularly noticeable when said photographic material is used as a color paper for direct viewing. Color papers and other examples of the silver halide photographic material of the present invention may be monochromatic or multicolored.

Silver halides that can be used in the silver halide photographic material of the present invention include silver bromide, silver iodobromide, silver iodochloride, silver chlorobromide, silver chloride and any other types that are customarily used in silver halide emulsions.

The silver halide emulsion to be used in the present invention may be chemically sensitized by any known technique such as sulfur sensitization, selenium sensitization, reduction sensitization or noble metal sensitization.

The silver halide emulsion to be used in the present invention may be optically sensitized to have sensitivity in a desired wavelength range using dyes that are known as spectral sensitizers in the art.

Gelatin is used advantageously as a binder (or protective colloid) in the silver halide photographic material of the present invention. Other hydrophilic colloids may also be used, such as gelatin derivatives, graft polymers of gelatin and other high-molecular weight compounds, proteins, sugar derivatives, cellulosic derivatives, and synthetic hydrophilic high-molecular weight materials such as homopolymers and copolymers.

Photographic emulsion layers and other hydrophilic colloidal layers in the silver halide photographic material of the present invention are hardened by using, either independently or in combination, those hardeners which crosslink the molecules of binders (or protective colloids) to increase the film strength. Hardeners are desirably added in amounts that are capable of hardening photographic materials to such an extent that there is no need to incorporate hardeners in processing solutions. If desired, hardeners may be incorporated in processing solutions.

The silver halide photographic material of the present invention may have uv absorbers contained in protective layers, inter mediates and other hydrophilic colloidal layers in order to prevent fogging due to the discharge of static buildup that occurs in the photographic material on account of triboelectrification or other phenomena, as well as to prevent image deterioration due to ultraviolet radiation.

The silver halide photographic material of the present invention may be provided with auxiliary layers such as a filter layer, an anti-halo layer and an anti-irradiation layer. These layers and/or emulsion layers may contain dyes that flow out of the color photographic material during development or which are bleachable.

Silver halide emulsion layers and/or other hydrophilic colloidal layers in the silver halide photographic material of the present invention may have matting agents incorporated therein in order to reduce the gloss of the photographic material, enhance its writability or to prevent one unit of the photographic material from sticking to another.

The silver halide photographic material of the present invention may have lubricants incorporated therein in order to reduce sliding friction.

The silver halide photographic material of the present invention may have antistats incorporated therein in order to prevent static buildup. Antistats may be incorporated in an anti static layer on the side of a support where no emulsion layers are provided, or they may be incorporated in emulsion layers and/or protective colloids on the side of the support where emulsion layers are provided.

Photographic emulsion layers and/or other hydrophilic colloidal layers in the silver halide photographic material of the present invention may incorporate various surfactants for achieving multiple purposes including improved coatability, prevention of static buildup, improved slip property, efficient emulsification and dispersion, anti-blocking and improved photographic characteristics such as accelerated development, contrastiness and increased sensitivity.

Photographic emulsion layers and other layers in the silver halide photographic material of the present invention are coated various supports including: flexible reflective supports such as baryta paper, paper laminated with α-olefinic polymers, paper supports that permit α-olefinic polymer layer to be readily released, and synthetic papers; reflective supports having white pigments coated on synthetic or semi-synthetic polymers such as cellulose acetate, cellulose nitrate, polystyrene, polyvinyl chloride, polyethylene terephthalate, polycarbonate and polyamide; and rigid supports such as glass, metal and ceramic sheets. Reflective supports as thin as 120 - 160 µm can also be used.

The supports to be used in the present invention may be of a reflection or transmission type. In order to impart reflectivity, white pigments may be incorporated in the supports or the latter may be coated with a hydrophilic colloidal layer containing a white pigment. White pigments may be inorganic or organic, with inorganic white pigments being preferred. Illustrative inorganic white pigments include alkaline earth metal sulfates such as barium sulfate, alkaline earth metal carbonates such as calcium carbonate, silicas such as fine particulate silicic acid and synthetic silicates, as well as calcium silicate, alumina, alumina hydrates, titanium oxide, zinc oxide, talc and clay. Barium sulfate and titanium oxide are preferred.

The support of the silver halide photographic material or the present invention may be subjected to surface treatments such as corona discharge, irradiation with ultraviolet rays and flame treatment before emulsion layers and other photographic layers are applied either directly or with one or more subbing layers being provided in order to improve various properties such as adhesion to the surface of the support, antistatic property, dimensional stability, friction resisting property, hardness, anti-halo property, and friction characteristics.

Thickeners may be used in order to improve the coatability of silver halide emulsions in the production of the silver halide photographic material of the present invention. Particularly advantageous coating methods are extrusion coating and curtain coating which are capable of simultaneous application of two or more layers.

Known color developing agents that are extensively used in various color photographic processes may be incorporated in color developing solutions for processing the silver halide photographic material of the present invention. The color developed photographic material of the present invention may be immediately processed with processing solutions having a bleaching capability; alternatively, it may be processed with a "bleach-fixing solution" which has both bleaching and fixing capabilities.

Metal complex salts of organic acids are typically used as bleaching agents in the bleaching step.

The following examples are provided for the purpose of further illustrating the present invention but are in no ways to be taken an limiting.

### Example 1

Paper supports each laminated with polyethylene on one side and with TiO₂ containing polyethylene on the other side were coated with seven layers (see below) to prepare samples of multi-layered silver halide color photographic material. The coating solutions for the seven layers were prepared in the following manner.

### Coating solution for the first layer:

A yellow coupler (26.7 g; see Table 2), 10.0 g of a dye image stabilizer (ST-1), 6.67 g of ST-2, 0.67 g of an anti-stain agent (HQ-1), 6.67 g of a high-boiling point organic solvent (DNP) and 60 ml of ethyl acetate were mixed to form a solution. The solution was emulsified and dispersed in 220 ml of a 10% aqueous solution of gelatin containing 7 ml of a 20% solution of surfactant (SU-1) by means of an ultrasonic: homogenizer, to thereby prepare a yellow coupler dispersion. This dispersion was mixed with a blue-sensitive silver halide emulsion (silver content, 8.67 g; for the method of its preparation, see below) to prepare the coating solution for the first layer.

The coating solutions for the second to the seventh layers were prepared in substantially the same manner. Preservatives were added as required.

The layer arrangement is shown in Table 1 below.

DOP dioctyl phthalate DNP dinonyl phthalate
DIDP diisodecyl phthalate PVP polyvinylpyrrolidone compound H-1 shown below was used as a hardener.

### Comparative compound A

### Preparation of blue-sensitive silver halide emulsion

Solutions A and B (see below) were added simultaneously over 30 minutes to 1,000 ml of a 2% aqueous solution of gelatin held at 40°C, with the pAg and pH being held at 6.5 and 3.0, respectively. Further, solutions C and D (see below) were added simultaneously over 180 minutes, with the pAg and pH being controlled at 7.3 and 5.5, respectively.

The pAg was controlled by the method described in Japanese Patent Application (kokai) No. 45437/1984 and the pH was controlled using an aqueous solution of sulfuric acid or sodium hydroxide.

### Solution A

| | |
|---|---|
| Sodium chloride | 3.42 g |
| Potassium bromide | 0.03 g |
| Water | to make 200 ml |

### Solution B

| | |
|---|---|
| Silver nitrate | 10 g |
| Water | to make 200 ml |

### Solution C

| | |
|---|---|
| Sodium chloride | 102.7 g |
| Potassium bromide | 1.0 g |
| Water | to make 600 ml |

### Solution D

| | |
|---|---|
| Silver nitrate | 300 g |
| Water | to make 600 ml |

After the addition of the four solutions, desalting was effected using a 5% aqueous solution of "Demol N" (Kao-Atlas Co., Ltd.) and a 20% aqueous solution of magnesium sulfate. The resulting dispersion was mixed with an aqueous solution of gelatin to prepare a monodispersed cubic emulsion EMP-1 having an average grain size of 0.85 µm, a variation coefficient (σ/r) of 0.07 and a AgCl content of 99.5 mol%.

The emulsion EMP-1 was chemically ripened with the following compounds at 50°C for 90 minutes to prepare a blue-sensitive silver halide emulsion (EmA).

| | |
|---|---|
| Sodium thiosulfate | 0.8 mg/mol AgX |
| Chloroauric acid | 0.5 mg/mol AgX |
| Stabilizer (SB-5) | 6 x 10⁻⁴ mol/mol AgX |
| Sensitizing dye (D-1) | 5 x 10⁻⁴ mol/mol AgX |

### Preparation of green-sensitive silver halide emulsion

The procedure for preparing EMP-1 was repeated except that the times over which solutions A/B and solutions C/D were added were varied. Thus, a monodispersed cubic emulsion EMP-2 was prepared: it had an average grain size of 0.43 µm, a variation coefficient (σ/r) of 0.08 and a AgCl content of 99.5 mol%.

The emulsion EMP-2 was chemically ripened with the following compounds at 55°C for 120 minutes to prepare a green-sensitive silver halide emulsion (EmB).

| | |
|---|---|
| Sodium thiosulfate | 1.5 mg/mol AgX |
| Chloroauric acid | 1.0 mg/mol AgX |
| Stabilizer (SB-5) | 6 x 10⁻⁴ mol/mol AgX |
| Sensitizing dye (D-2) | 4 x 10⁻⁴ mol/mol AgX |

### Preparation of red-sensitive silver halide emulsion

The procedure for preparing EMP-1 was repeated except that the times over which solutions A/B and solutions C/D were added were varied. Thus, a monodispersed cubic emulsion EMP-3 was prepared; it had an average grain size or 0.50 µm, a variation coefficient (σ/r) of 0.08 and a AgCl content of 99.5 mol%.

The emulsion EMP-3 was chemically ripened with the following compounds at 60°C for 90 minutes to prepare a red-sensitive silver halide emulsion (EmC).

| | |
|---|---|
| Sodium thiosulfate | 1.8 mg/mol AgX |
| Chloroauric acid | 2.0 mg/mol AgX |
| Stabilizer (SB-5) | 6 x 10⁻⁴ mol/mol AgX |
| Sensitizing dye (D-3) | 8.0 x 10⁻⁴ mol/mol AgX |

The samples thus prepared were exposed in the usual manner and processed by the following scheme.

| Steps | Temperature (°C) | Time (SEC) |
|---|---|---|
| Color development | 35.0 ± 0.3 | 45 |
| Bleach-fixing | 35.0 ± 0.5 | 45 |
| Stabilization | 30 - 34 | 90 |
| Drying | 60 - 80 | 60 |

### Color developing solution

| | |
|---|---|
| Pure water | 800 ml |
| Triethanolamine | 10 g |
| N,N-Diethylhydroxylamine | 5 g |
| Potassium bromide | 0.02 g |
| Potassium chloride | 2 g |
| Potassium sulfite | 0.3 g |
| 1-Hydroxyethylidene-1,1-diphosphonic acid | 1.0 g |
| Ethylenediaminetetraacetic acid | 1.0 g |
| Catechol-3,5-diphosphonic acid disodium salt | 1.0 g |
| N-Ethyl-N -β-methanesulfonamidoethyl-3-methyl-4-aminoaniline sulfate | 4.5 g |
| Optical brightening agent (4,4'-diaminostilbene disulfonic acid derivative) | 1.0 g |
| Potassium carbonate | 27 g |
| Water | to make 1.000 ml |
| pH | adjusted to 10.10. |

### Bleach-fixing solution

| | |
|---|---|
| Ethylenediaminetetraacetic acid iron (II) ammonium dihydrate | 60 g |
| Ethylenediaminetetraacetic acid | 3 g |
| Ammonium thiosulfate (70% aq. sol.) | 100 ml |
| Ammonium thiosulfate (40% aq. sol.) | 27.5 ml |
| Water | to make 1,000 ml |
| pH | adjusted to 5.7 with potassium carbonate or glacial acetic acid |

### Stabilizing solution

| | |
|---|---|
| 5-Chloro-2-methyl-4-isothiazolin-3-one | 1.0 g |
| Ethylene glycol | 1.0 g |
| 1-Hydroxyethylidene-1,1-diphosphonic acid | 2.0 g |
| Ethylenediaminetetraacetic acid | 1.0 g |
| Ammonium hydroxide (20% aq. sol.) | 3.0 g |
| Optical brightening agent (4.4'-diaminostilene disulfonic acid derivative) | 1.5 g |
| Water | to make 1,000 ml |
| pH | adjusted to 7.0 with sulfuric acid or potassium hydroxide |

### Evaluation

The processed samples were subjected to various evaluation tests by the following methods and the results are shown in Table 3.

### Sensitivity of blue-sensitive layer:

The photographic sensitivity that provided a blue optical density of 0.8 was determined in relative terms, with the value for sample No. 1 being taken as 100. Variation in the sensitivity of raw stock in storage:

The samples were stored in a test bath at 50°C and 50% r.h. for 7 days and the percent reduction in the sensitivity of blue-sensitive layer was determined.$\text{Sensitivity reduction} \left(\text{%}\right) \text{=} \frac{\text{sensitivity before storage - sensitivity after storage}}{\text{sensitivity before storage}} \text{x 100}$

### Color reproduction:

A picture of color chart was taken on a commercial color film (GX-II 100 of Konica Corp.) and prints of the samples were prepared using the developed negative films and the color reproduction on each print was evaluated visually. The results were evaluated by the following criteria:
o , excellent
Δ , acceptable
x , poor

**Table 3**

| Sample No. | Sensitivity of blue-sensitive layer | Reduction(%) in the sensitivity of blue-sensitive layer during storage | Color reproduction | Remarks |
|---|---|---|---|---|
| 1 | 100 | 10 | x | comparison |
| 2 | 100 | 9 | x | do. |
| 3 | 105 | 25 | o | do. |
| 4 | 105 | 21 | o | do. |
| 5 | 104 | 26 | o | do. |
| 6 | 105 | 25 | o | do. |
| 7 | 106 | 9 | o | invention |
| 8 | 105 | 8 | o | do. |
| 9 | 104 | 7 | o | do. |
| 10 | 107 | 8 | o | do. |
| 11 | 103 | 9 | o | do. |
| 12 | 106 | 7 | o | do. |
| 13 | 104 | 10 | o | do. |
| 14 | 104 | 6 | o | do. |
| 15 | 106 | 7 | o | do. |
| 16 | 103 | 8 | o | do. |
| 17 | 103 | 10 | o | do. |

As is clear from Table 3, the samples of the present invention achieved good color reproduction; furthermore, they experienced substantially small reduction in the sensitivity of blue-sensitive layer when they were stored as raw stock.

### Example 2

Additional samples were prepared as in Example 1 except that the following AgClBr emulsions were used as blue-, green- and red-sensitive emulsions.

### Blue-sensitive AgClBr emulsion:

A AgClBr emulsion having an average grain size of 0.7 µm and a AgBr content of 90 mol% was subjected to optimum sensitization with sodium thiosulfate at 57°C, and a sensitizing dye (D-1) and astabilizing agent (Z-1) were added,

### Green-sensitive AgClBr emulsion:

A AgClBr emulsion having an average grain size of 0.5 µm and a AgBr content of 70 mol% was subjected to optimum sensitization with sodium thiosulfate at 57°C, and a sensitizing dye (D-2) and a stabilizer (Z-1) were added.

### Red-sensitive AgClBr emulsion:

A AgClBr emulsion having an average grain size of 0.4 µm and a AgBr content of 60 mol% was subjected to optimum sensitization with sodium thiosulfate, a sensitizing dye (D-3) and a phenolic resin at 60°C, and a stabilizer (Z-1) was added.

The samples thus prepared were exposed in the usual manner and processed by the following scheme.

| Steps | Temperature, °C | Time, sec |
|---|---|---|
| Color development | 38 | 210 |
| Bleach-fixing | 33 | 90 |
| Washing | 25 - 30 | 180 |
| Drying | 75 - 80 | ca. 120 |

### Processing solution formulas

### Bleach-fixing solution:

| | |
|---|---|
| Ethylenediaminetetraacetic acid iron (II) ammonium dihydrate | 60 g |
| Ethylenediaminetetraacetic acid | 3 g |
| Ammonium thiosulfate (70% aq. sol.) | 100 ml |
| Ammonium sulfite (40% aq. sol.) | 27.5 ml |
| Water | to make 1,000 ml |
| pH | adjusted to 7.1 with potassium carbonate or glacial acetic acid |

The samples prepared in accordance with the present invention were satisfactory in terms of both raw stock stability and color reproduction.

### Example 3

Direct positive-acting samples were prepared by the method described below and subjected to the same evaluations as in Example 1.

### Preparation of emulsion EM-1

An solution of silver nitrate and an aqueous solution containing potassium bromide and sodium chloride in a KBr to NaCl molar ratio of 40:60 were added simultaneously by a controlled double-jet method to an aqueous solution containing ossein gelatin with vigorous stirring at a controlled temperature of 55°C, thereby obtaining a cubic AgClBr emulsion A having an average grain size of 0.3 µm. Using the grains in emulsion A as core grains, an aqueous solution of silver nitrate and an aqueous solution of sodium chloride were added simultaneously by a double-jet method with the temperature and pAg being controlled ad 55°C and 6, respectively, thereby obtaining a cubic monodispersed core/shell emulsion EM-1 having an average grain size of 0.6 µm (the spread of grain size distribution* was 8%).
$\text{* Spread of grain size distribution (%) =} \frac{\text{standard deviation of grain size}}{\text{average grain size}} \text{× 100}$

### Composition of light-sensitive layers

The components of the individual photographic layers are shown below, with the coat weight being expressed by g/m. For silver halides, the coat weight is expressed in terms of silver.

### First layer (red-sensitive layer)

### Second layer (intermediate layer)

| | |
|---|---|
| Gelatin | 0.75 |
| Anti-color mixture agent (HQ-1) | 0.06 |
| Solvent (DOP) | 0.07 |

### Third layer (green-sensitive layer)

| | |
|---|---|
| Green-sensitive emulsion prepared by spectral sensitization after addition of green-sensitive sensitizing dye (GD-1) to EM-1 | 0.27 |
| Gelatin | 1.3 |
| Magenta coupler (M-23) | 0.24 |
| Image stabilizer (ST-3) | 0.20 |
| Solvent (DOP) | 0.32 |

### Fourth layer (intermediate layer)

### Same as the second layer

### Fifth layer (yellow filter layer)

### Sixth layer (anti-color mixture layer)

| | |
|---|---|
| Gelatin | 0.40 |
| Anti-color mixture agent (HQ-1) | 0.03 |
| Solvent (DOP) | 0.04 |

### Seventh layer (blue-sensitive layer)

| | |
|---|---|
| Blue-sensitive emulsion prepared by spectral sensitization after addition of blue-sensitive sensitizing dye (BD-1) to EM-1 | 0.50 |
| Gelatin | 1.35 |
| Yellow coupler (Y-6) | 0.90 |
| Image stabilizer (ST-1) | 0.30 |
| Solvent (DNP) | 0.20 |
| Preservative (9) | 1 x 10⁻³ |

### Eighth layer (uv absorbing layer)

| | |
|---|---|
| Gelatin | 0.54 |
| UV absorber (UV-1) | 0.10 |
| UV absorber (UV-2) | 0.28 |
| Solvent (DNP) | 0.12 |

### Ninth layer (protective layer)

| | |
|---|---|
| Gelatin | 0.12 |
| Preservative (9) | 1 x 10⁻³ |

### Processing scheme

| Steps | Time, sec | Temperature, °C |
|---|---|---|
| Immersion | 2 | 38 |
| Exposure | 5 | 38(1 lux) |
| Development | 25 | 38 |
| Bleach-fixing | 45 | 35 |
| Stabilization | 90 | 25 - 30 |
| Drying | 45 | 75 - 80 |

### Processing solutions

### Color developing solution:

### Bleach-fixing solution:

| | |
|---|---|
| Diethylenetriaminepentaacetic acid iron (II) ammonium salt | 90 g |
| Diethylenetriaminepentaacetic acid | 3 g |
| Ammonium thiosulfate (70% aq. sol.) | 180 ml |
| Ammonium sulfite (40% aq. sol.) | 27.5 ml |
| 3-Mercapto-1,2,4-triazole | 0.15 g |
| Water | to make 1,000 ml |
| pH | adjusted to 7.1 with potassium carbonate or glacial acetic acid |

### Stabilizing solution:

The samples prepared in accordance with the present invention were satisfactory in terms of both raw stock stability and color reproduction.

As will be apparent from the foregoing description, the present invention provides a silver halide photographic material that achieves faithful color reproduction and which yet has good raw stock stability.

## Claims

1. A silver halide color photographic material comprising a support having provided thereon a yellow coupler represented by formula (Y-I), a magenta coupler represented by formula (M-I) and a cyan coupler represented by formula (C-I, wherein the photographic material further comprises at least one of the compounds represented by formulae (I), (II), (III) and (IV): where R₁ is an alkyl group, a cycloalkyl group or an aryl group; R₂ is an alkyl group, a cycloalkyl group, an aryl group or an acyl group; R₃ is an optional substituent on the benzene ring; n is 0 or 1; X₁ is a group capable of leaving upon coupling with the oxidation product of a developing agent; and Y₁ is an organic group; where Z is the nonmetallic group necessary to form a nitrogenous hetero ring which may optionally have a substituent; X is a hydrogen atom or a group capable of leaving upon reaction with the oxidation product of a color developing agent; and R is a hydrogen atom or a substituent; where R₁₁ is a ballast group; R₁₂ is an alkyl group having 2 or more carbon atoms; and Z₁ is a hydrogen atom or an atom or group that is capable of leaving upon reaction with the oxidation product of a color developing agent; where R₁₀ is a lower alkylene group; M is a hydrogen atom, an alkali metal or an alkyl group; X is a halogen atom, an alkyl group, a cycloalkyl group, an aryl group, a carboxyl group, an amino group, a hydroxyl group, a sulfo group, a nitro group or an alkoxycarbonyl group; n is 0 or 1; and m is an integer of 1 - 5 ; where R₂₀ is a hydrogen atom, an alkyl group, a cycloalkyl group, an alkenyl group, an aralkyl group, an aryl group, an alkoxy group, -CONHR (R is an alkyl, aryl, alkylthio, arylthio, alkylsulfonyl or arylsulfonyl group) or a heterocyclic group; R₃₀ and R₄₀ are each a hydrogen atom, a halogen atom, an alkyl group, a cycloalkyl group, an aryl group, a heterocyclic group, a cyano group, an alkylthio group, an arylthio group, an alkylsulfoxide group, an alkylsulfonyl group, or an alkylsulfinyl group, provided that R₃₀ and R₄₀ may combine together to form an optionally substituted benzene ring; where R₅₀ and R₆₀ are each a hydrogen atom, a halogen atom, a lower alkyl group having 1 - 5 carbon atoms or a hydroxymethyl group; and R₇₀ is a hydrogen atom or a lower alkyl group having 1 - 5 carbon atoms; where R₈₀ is a hydrogen atom, an alkyl group or an aryl group; R₉₀ is a hydrogen atom, an alkyl group, an aryl group, a nitro group, a carboxyl group, a sulfo group, a sulfamoyl group, a hydroxy group, a halogen atom, an alkoxy group or a thiazolyl group; m is 0 or 1; and Z is the atomic group necessary to form a thiazolyl ring.

2. A photographic material according to claim 1 wherein the yellow coupler represented by the general formula (Y-I) is n compound represented by the following general formula (Y-V): where R₁, R₂, R₃, X₁ and n have the same meanings as R₁, R₂,R₃, X₁ and n in the general formula (Y-I); J is or (where R₅ is a hydrogen atom, an alkyl group, an aryl group or a heterocyclic group); R₇ is an alkylene group, an arylene group, an alkylenearylene group, an arylenealkylene group or -A-V₁-B (where A and B are each an alkylene group, an arylene group, an alkylenearylene group or an arylenealkylene group; and V₁ is a divalent linkage group); R₈ is an alkyl group, a cycloalkyl group, an aryl group or a heterocyclic group; and P is a bonding group having a carbonyl or sulfonyl unit.

3. A photographic material according to claims 1 or 2, wherein the magenta coupler represented by the general formula (M-I) is a compound represented by the following general formula (M-II): where R₁, R₂ and X have the same meanings as R and X in the general formula (M-I).

4. A photographic material according to claims 1 to 3, wherein R₁₂ in the general formula (C-I) is an alkyl group having 2-6 carbon atoms and R₁₁ is a group represented by (where Rₙ₁ is an alkyl group having 1-12 carbon atoms, and Ar is an aryl group).

5. A photographic material according to any preceding claim, wherein the compounds represented by the general formulae (I), (II), (III) and (IV) are used in amounts ranging from 1 x 10⁻⁴ to 1 x 10⁻ g/m.

6. A photographic material according to any preceding claim, wherein a high-boiling point organic solvent is used in dissolving dye-forming couplers and other compounds.

7. A photographic material according to claim 6 wherein said high-boiling point organic solvent is chosen from esters, amides, ketones and hydrocarbon compounds that have dielectric constants of no more than 6.5.

8. A photographic material according to any preceding claim, which is a color paper for use in direct viewing.

## Patentansprüche

1. Farbphotographisches Silberhalogenid-Aufzeichnungsmaterial mit einem Schichtträger und einem darauf befindlichen Gelbkuppler der Formel (Y-I), Purpurrotkuppler der Formel (M-I) und Blaugrünkuppler der Formel (C-I), welches zusätzlich mindestens.eine Verbindung der Formeln (I), (II), (III) und (IV) enthält: worin bedeuten:
R₁ eine Alkylgruppe, eine Cycloalkylgruppe oder eine Arylgruppe;
R₂ eine Alkylgruppe, eine Cycloalkylgruppe, eine Arylgruppe oder eine Acylgruppe;
R₃ einen möglichen Substituenten am Benzolring; n = 0 oder 1;
X₁ eine bei der Kupplung mit dem Oxidationsprodukt einer Entwicklerverbindung abspaltbare Gruppe und
^{Y}₁ eine organische Gruppe; worin bedeuten:
Z diejenige nichtmetallische Gruppe, die zur Bildung eines gegebenenfalls substituierten stickstoffhaltigen Heterorings erforderlich ist;
X ein Wasserstoffatom oder eine bei der Reaktion mit dem Oxidationsprodukt einer Farbentwicklerverbindung abspaltbare Gruppe und
R ein Wasserstoffatom oder einen Substituenten; worin bedeuten:
R₁₁ eine Ballastgruppe;
R₁₂ eine Alkylgruppe mit 2 oder mehr Kohlenstoffatomen und
Z₁ ein Wasserstoffatom oder ein(e) bei der Reaktion mit dem Oxidationsprodukt einer Farbentwicklerverbindung abspaltbare(s) Atom oder Gruppe; worin bedeuten:
R₁₀ eine Niedrigalkylengruppe;
M ein Wasserstoffatom, ein Alkalimetall oder eine Alkylgruppe;
X ein Halogenatom, eine Alkylgruppe, eine Cycloalkylgruppe, eine Arylgruppe, eine Carboxylgruppe, eine Aminogruppe, eine Hydroxylgruppe, eine Sulfogruppe, eine Nitrogruppe oder eine Alkoxycarbonylgruppe;
n = 0 oder 1 und
m eine ganze Zahl von 1 bis 5; worin bedeuten:
R₂₀ ein Wasserstoffatom, eine Alkylgruppe, eine Cycloalkylgruppe, eine Alkenylgruppe, eine Aralkylgruppe, eine Arylgruppe, eine Alkoxygruppe, -CONHR mit R gleich einer Alkyl-, Aryl-, Alkylthio-, Arylthio-, Alkylsulfonyl- oder Arylsulfonylgruppe oder eine heterocyclische Gruppe und
R₃₀ und R₄₀ jeweils ein Wasserstoffatom, ein Halogenatom, eine Alkylgruppe, eine Cycloalkylgruppe, eine Arylgruppe, eine heterocyclische Gruppe, eine Cyanogruppe, eine Alkylthiogruppe, eine Arylthiogruppe, eine Alkylsulfoxidgruppe, eine Alkylsulfonylgruppe oder eine Alkylsulfinylgruppe, wobei R₃₀ und R₄₀ zusammen auch einen gegebenenfalls substituierten Benzolring bilden können; worin bedeuten:
R₅₀ und R₆₀ jeweils ein Wasserstoffatom, ein Halogenatom, eine Niedrigalkylgruppe mit 1 bis 5 Kohlenstoffatom(en) oder eine Hydroxymethylgruppe und R₇₀ ein Wasserstoffatom oder eine Niedrigalkylgruppe mit 1 bis 5 Kohlenstoffatom(en); worin bedeuten:
R₈₀ ein Wasserstoffatom, eine Alkylgruppe oder eine Arylgruppe;
R₉₀ ein Wasserstoffatom, eine Alkylgruppe, eine Arylgruppe, eine Nitrogruppe, eine Carboxylgruppe, eine Sulfogruppe, eine Sulfamoylgruppe, eine Hydroxygruppe, eine Halogenatom, eine Alkoxygruppe oder eine Thiazolylgruppe;
m = 0 oder 1 und
Z die zur Bildung eines Thiazolylrings erforderliche Atomgruppe.

2. Photographisches Aufzeichnungsmaterial nach Anspruch 1, wobei es sich bei dem Gelbkuppler der allgemeinen Formel (Y-I) um eine Verbindung der folgenden allgemeinen Formel (Y-V) handelt: worin R₁, R₂, R₃, X₁ und n die Bedeutung von R₁, R₂, R₃, X₁ und n in der allgemeinen Formel (Y-I) aufweisen,
J für mit R₅ gleich einem Wasserstoffatom, einer Alkylgruppe, einer Arylgruppe oder einer heterocyclischen Gruppe steht;
R₇ eine Alkylengruppe, eine Arylengruppe, eine Alkylenarylengruppe, eine Arylenalkylengruppe oder -A-V₁-B mit A und B jeweils gleich einer Alkylengruppe, Arylengruppe, Alkylenarylengruppe oder Arylenalkylengruppe und V₁ gleich einer zweiwertigen verbindenden Gruppe darstellt;
R₈ einer Alkylgruppe, Cycloalkylgruppe, Arylgruppe oder heterocyclischen Gruppe entspricht und P eine verbindende Gruppe mit einer Carbonyl- oder Sulfonyleinheit bedeutet.

3. Photographisches Aufzeichnungsmaterial nach Anspruch 1 oder 2, wobei es sich bei dem Purpurrotkuppler der allgemeinen Formel (M-I) um eine Verbindung der folgenden allgemeinen Formel (M-II): worin R₁, R₂ und X die Bedeutung von R und X in der allgemeinen Formel (M-I) aufweisen, handelt.

4. Photographisches Aufzeichnungsmaterial nach Ansprüchen 1 bis 3, wobei R₁₂ in der allgemeinen Formel (C-I) für eine Alkylgruppe mit 2 bis 6 Kohlenstoffatomen steht und R₁₁ eine Gruppe mit Rₙ₁ gleich einer Alkylgruppe mit 1 bis 12 Kohlenstoffatom(en) und Ar gleich einer Arylgruppe bedeutet.

5. Photographisches Aufzeichnungsmaterial nach einem der vorhergehenden Ansprüche, wobei die Verbindungen der allgemeinen Formeln (I), (II), (III) und (IV) in Mengen von 1 x 10⁻⁴ bis 1 x 10⁻ g/m eingesetzt sind.

6. Photographisches Aufzeichnungsmaterial nach einem der vorhergehenden Ansprüche, wobei zum Auflösen farbstoffbildender Kuppler und sonstiger Verbindungen ein hochsiedendes organisches Lösungsmittel verwendet wird.

7. Photographisches Aufzeichnungsmaterial nach Anspruch 6, wobei das hochsiedende organische Lösungsmittel aus Estern, Amiden, Ketonen und Kohlenwasserstoffverbindungen mit Dielektrizitätskonstanten von nicht mehr als 6,5 ausgewählt ist.

8. Photographisches Aufzeichnungsmaterial nach einem der vorhergehenden Ansprüche, bei welchem es sich um ein Farbpapier zur direkten Betrachtung handelt.

## Revendications

1. Matériau photographique couleur à l'halogénure d'argent, comprenant un support ayant, sur celui-ci, un agent de couplage jaune représenté par la formule (Y-I), un agent de couplage magenta représenté par la formule (M-I) et un agent de couplage cyan représenté par la formule (C-I) où le matériau photographique comprend en outre au moins un des composés représentés par les formules (I), (II), (III) et (IV) : où R₁ est un groupe alkyle, un groupe cycloalkyle ou un groupe aryle ; R₂ est un groupe alkyle, un groupe cycloalkyle, un groupe aryle ou un groupe acyle ; R₃ est un substituant facultatif sur le cycle benzènique ; n est 0 ou 1; X₁ est un groupe capable de partir par couplage avec le produit d'oxydation d'un agent de développement ; et Y₁ est un groupe organique : où Z est le groupe non métallique nécessaire pour former un hétérocycle azoté qui peut facultativement avoir un substituant ; X est un atome d'hydrogène ou un groupe capable de partir par réaction avec le produit d'oxydation d'un agent de développement couleur ; et R est un atome d'hydrogène ou un substituant : où R₁₁ est un groupe ballast ; R₁₂ est un groupe alkyle ayant 2 atomes de carbone ou plus ; et Z₁ est un atome d'hydrogène ou un atome ou groupe qui est capable de partir par réaction avec le produit d'oxydation d'un agent de développement couleur : où R₁₀ est un groupe alkylène inférieur ; M est un atome d'hydrogène, un métal alcalin ou un groupe alkyle ; X est un atome d'halogène, un groupe alkyle, un groupe cycloalkyle, un groupe aryle, un groupe carboxyle, un groupe amino, un groupe hydroxyle, un groupe sulfo, un groupe nitro ou un groupe alcoxycarbonyle ; n est 0 ou 1 ; et m est un nombre entier de 1 à 5 : où R₂₀ est un atome d'hydrogène, un groupe alkyle, un groupe cycloalkyle, un groupe alcényle, un groupe aralkyle, un groupe aryle, un groupe alcoxy, un groupe -CONHR (R est un groupe alkyle, aryle, alkylthio, arylthio, alkylsulfonyle ou arylsulfonyle) ou un groupe hétérocyclique ; R₃₀ et R₄₀ sont chacun un atome d'hydrogène, un atome d'halogène, un groupe alkyle, un groupe cycloalkyle, un groupe aryle, un groupe hétérocyclique, un groupe cyano, un groupe alkylthio, un groupe arylthio, un groupe alkylsulfoxyde, un groupe alkylsulfonyle ou un groupe alkylsulfinyle, à condition que R₃₀ et R₄₀ puissent se combiner ensemble pour former un cycle benzènique éventuellement substitué : où R₅₀ et R₆₀ sont chacun un atome d'hydrogène, un atome d'halogène, un groupe alkyle inférieur ayant 1 à 5 atomes de carbone ou un groupe hydroxyméthyle ; et R₇₀ est un atome d'hydrogène ou un groupe alkyle inférieur ayant 1 à 5 atomes de carbone : où R₈₀ est un atome d'hydrogène, un groupe alkyle ou un groupe aryle ; R₉₀ est un atome d'hydrogène, un groupe alkyle, un groupe aryle, un groupe nitro, un groupe carboxyle, un groupe sulfo, un groupe sulfamoyle, un groupe hydroxy, un atome d'halogène, un groupe alcoxy ou un groupe thiazolyle ; m est 0 ou 1; et Z est le groupe atomique nécessaire pour former un cycle thiazolyle.

2. Matériau photographique selon la revendication 1, dans lequel l'agent de couplage jaune représenté par la formule générale (Y-I) est un composé représenté par la formule générale (Y-V) suivante : où R₁, R₂, R₃, X₁ et n ont les mêmes significations que R₁, R₂, R₃, X₁ et n dans la formule générale (Y-I) ;
J est (où R₅ est un atome d'hydrogène,
un groupe alkyle, un groupe aryle ou un groupe hétérocyclique) ; R₇ est un groupe alkylène, un groupe arylène, un groupe alkylènearylène, un groupe arylènealkylène ou -A-V₁-B (où A et B sont chacun un groupe alkylène, un groupe arylène, un groupe alkylènearylène ou groupe arylènealkylène ; et V est un groupe à liaison bivalente) ; R₈ est un groupe alkyle, un groupe cycloalkyle, un groupe aryle ou un groupe hétérocyclique ; et P est un groupe de liaison ayant une unité carbonyle ou sulfonyle.

3. Matériau photographique selon les revendications 1 ou 2, dans lequel l'agent de couplage magenta représenté par la formule générale (M-I) est un composé représenté par la formule générale (M-II) suivante : où R₁, R₂ et X ont les mêmes significations que R et X dans la formule générale (M-I).

4. Matériau photographique selon les revendications 1 à 3, dans lequel R₁₂ dans la formule générale (C-I) est un groupe alkyle ayant 2 à 6 atomes de carbone et R₁₁ est un groupe représenté par (où Rₙ₁ est un groupe alkyle ayant 1 à 12 atomes de carbone, et Ar est un groupe aryle).

5. Matériau photographique selon une quelconque revendication précédente, dans lequel les composés représentés par les formules générales (I), (Il), (III) et (IV) sont utilisés en des quantités allant de 1 x 10⁻⁴ à 1 x 10⁻ g/m.

6. Matériau photographique selon une quelconque revendication précédente, dans lequel un solvant organique à haut point d'ébullition est utilisé dans la dissolution des agents de couplage formant un colorant et d'autres composés.

7. Matériau photographique selon la revendication 6, dans lequel ledit solvant organique à haut point d'ébullition est choisi parmi les esters, amides, cétones et composés hydrocarbonés qui ont des constantes diélectriques non supérieures à 6,5.

8. Matériau photographique selon une quelconque revendication précédente, qui est un papier couleur pour utilisation dans le visionnage direct.
